

April 29, 1952

J. ROCKOFF

2,594,348

RUBBER COVERED ROLL

Filed Jan. 18, 1947

FIG. 1.



FIG. 2.



FIG. 3.



INVENTOR  
JOSEPH ROCKOFF  
BY  
Toulmin & Toulmin  
ATTORNEYS

## UNITED STATES PATENT OFFICE

2,594,348

## RUBBER COVERED ROLL

Joseph Rockoff, Dayton, Ohio, assignor to The Dayton Rubber Company, a corporation of Ohio

Application January 18, 1947, Serial No. 722,802

3 Claims. (Cl. 154—43)

1

This invention deals with coverings for rolls, in particular for rolls used for offset printing and textile machinery such as slasher rolls. Sponge rubber in such rolls is new, and in particular the use of a very thin sponge layer thereon. The sponge rubber provides for a good liquid control action and also for a high absorptive capacity both of which are essential in the case of offset printing rolls, such as form dampers and damper ductors used on offset lithographic presses and slasher rolls.

It is an object of this invention to provide coverings for rolls which are made of sponge rubber with a very fine and uniform texture.

It is another object of this invention to provide coverings for rolls which show a high degree of porosity.

It is another object of this invention to provide coverings for rolls which, in spite of the high degree of porosity, are of considerable stability and rigidity so that deformation during operation does not occur.

It is still another object of this invention to provide coverings for rolls which have an extremely long service life.

It is still another object of this invention to provide coverings for rolls which have a high absorptive capacity for liquids.

It is still another object of this invention to provide coverings for slasher rolls with which the amount of sizing material on the yarn may be controlled easily.

It is still another object of this invention to provide coverings for rolls from sponge rubber which may be thoroughly cleaned without difficulty.

These and other objects are accomplished by constructing a roll covering so that it has an inner bulk layer of solid rubber or rubber-like material and a more or less thin surface layer of sponge rubber with fine interconnected pores of uniform size.

The invention will be more fully understood from the following description taken in connection with the accompanying drawings, in which:

Figure 1 is a perspective view of a roll covering of my invention as mounted on an axle shaft;

Figure 2 is a longitudinal section taken along line 2—2 of Figure 1; and

Figure 3 is an enlarged fragmentary longitudinal section from which the shape and arrangement of the pores is more clearly recognizable.

Referring to the drawings in detail, the reference numeral 4 indicates an axle shaft on which

2

a covering, generally designated with 5, is mounted. This covering 5 comprises an inner bulk layer 6 made of solid rubber or rubberlike material and an outer thinner sponge layer 7. It is obvious (Fig. 3) that the outer sponge layer 7 consists of rubber material 8 and pores 9 uniformly distributed therein. These pores 9 are interconnected and of relatively regular size. This feature of the pores being interconnected is of the utmost importance, since by this the efficiency of the roll covering is greatly enhanced. Even the pores located at the innermost layer of the sponge section are accessible to the material to be treated and consequently the absorptive capacity of the entire unit is increased.

The covering of my invention is made by first arranging solid rubber material onto a mandrel in a thickness desired of the bulk rubber layer, vulcanizing said layer, thereafter preparing a mixture of rubber, or rubberlike material, and crystals of a water soluble salt and applying said mixture over said solid rubber layer. The built-up unit is then again vulcanized, preferably after being wrapped in a wet cloth whereby the layers become integrally united. After vulcanization, the cover is ground to the precise size and surface condition desired. Thereafter the salt is removed by leaching it out with water. This leaching process is preferably carried out under pressure, for example under a pressure of approximately 200 lbs. per square inch. In order to obtain, after leaching, pores that are interconnected and thus to make possible that the surface layer in its entire thickness may be utilized, a relatively great amount of salt crystals is incorporated into said surface layer. It is evident that the degree of porosity may be adjusted by merely varying the amount of salt added. I have obtained very satisfactory results with 200 to 300 parts by weight of salt per 100 parts of rubber or rubberlike material, but it will be understood that the particular proportions of salt and rubber are widely variable depending upon the texture.

Instead of grinding the surface prior to leaching, the salt crystals may also be removed first and then the covering be surface-conditioned by grinding. In this case it is advantageous, though not obligatory, to dry the unit prior to grinding.

The method of manufacturing the roll coverings described forms the subject of my co-pending application Serial No. 722,804, filed January 18, 1947, now Patent No. 2,500,573 granted March 14, 1950.

Various kinds of rubber materials are usable

for the object of my invention. Natural as well as synthetic rubbers are operative, the selection being dependent upon the use intended for the covering. Synthetic rubbers which were found satisfactory for my purpose are the neoprenes, butadiene copolymers, such as butadiene acrylonitrile copolymer and butadiene styrene copolymer, and the polysulfide rubbers known under the trade-name Thiokol. Filler materials, vulcanizing agents and other auxiliary substances known may be added to the rubber materials. The term rubber as used herein therefore includes natural rubber as well as synthetic rubberlike materials of the types represented by the chloroprene polymers, such as Neoprene; butadiene copolymers, such as butadiene-acrylonitrile and butadiene-styrene; and the polysulfide rubbers, such as "Thiokol."

As the pore-creating salt, any water soluble salt is usable which does not decompose or disintegrate at the vulcanization temperature. For instance, sodium chloride, various kinds of sulfates, sugar and others obvious to those skilled in the art may be used.

It will be understood that the thickness of the outer sponge layer is dependent upon the size of the covering and upon the purpose for which it is intended. In the case of slasher rolls, a thickness of 1 to 2 inches was preferred for the bulk layer and of  $\frac{1}{2}$  to  $\frac{3}{4}$  of an inch for the finished outer layer. Similarly the hardness of the material also has to be adjusted according to the purpose intended. A hardness of from 40 to 60 on the Shore scale A was found the optimal range for slasher rolls.

In the following one example which was found very satisfactory for the roll of my invention is given without the intention of limiting the invention thereto.

#### Example

##### (a) Compound for the inner bulk layer:

|                                      |                                                   |
|--------------------------------------|---------------------------------------------------|
| 100 parts by weight neoprene type GN | 5 parts by weight zinc oxide                      |
| 10 parts by weight cumar resin       | 5 parts by weight rosin oil                       |
| 10 parts by weight mineral oil       | 10 parts by weight light calcined magnesium oxide |
| 50 parts by weight factice           | 1 part by weight Agerite (parabenzyloxy phenol)   |

##### (b) Compound for the sponge layer:

|                                                   |    |
|---------------------------------------------------|----|
| 100 parts by weight neoprene type GN              | 55 |
| 30 parts by weight clay                           |    |
| 1 part by weight Agerite powder                   |    |
| 0.50 part by weight benzothiazyl disulfide        |    |
| 15 parts by weight mineral oil                    |    |
| 10 parts by weight light calcined magnesium oxide | 60 |
| 10 parts by weight zinc oxide                     |    |
| 300 parts by weight crystalline sodium chloride   |    |

It will be obvious that by the specific method of preparing the sponge rubber layer on the coverings of my invention an article is obtained which has an extremely uniform texture and in which the holes are interconnected. These interconnected holes or pores form channel-like voids which have a considerably higher suction

than have small individual pores; as a result thereof a greater absorbability is obtained. Due to the inner solid bulk layer, the rigidity and form-stability of the covering are considerably greater than if it were made entirely of sponge rubber. This feature of having only the outer layer made of sponge rubber facilitates cleaning of the channels in case this should become necessary, since the innermost ends of the channels are better accessible to the cleaning means. Furthermore, due to the uniform size and distribution of the cavities, the operation of the covering is more uniform at its various locations.

It will be understood that although a number of uses for the articles of my invention have been set forth, these represent merely examples, since there are a great many other possibilities for which the invention is, or might become, of value.

It will also be understood that while there have been described herein certain specific embodiments of my invention, it is not intended thereby to have it limited to or circumscribed by the specific details given in view of the fact that this invention is susceptible to various modifications and changes which come within the spirit of this disclosure and the scope of the appended claims.

I claim:

1. A rubber covered roll for the application of liquid materials having substantial stability and resistance to deformation during use, and having a surface possessed of a high degree of porosity, a uniform texture, and a high absorptive capacity for liquids, which comprises a shaft, a solid inner bulk rubber layer surrounding said shaft and mounted thereon, and an outer sponge rubber layer surrounding and integrally united with said inner layer, said outer layer being of less thickness than the inner layer, said outer layer having uniformly distributed therethrough a multitude of channels formed of interconnected uniformly distributed minute pores, said pores conforming in shape to granules of finely divided water soluble material incorporated in said outer layer in the proportion of at least twice as much soluble material by weight as rubber and removed therefrom by leaching.

2. A rubber covered roll according to claim 1 wherein the water soluble material is crystalline sodium chloride.

3. A rubber covered roll according to claim 1 wherein the outer layer is composed of a butadiene copolymer type of synthetic rubber.

JOSEPH ROCKOFF.

#### REFERENCES CITED

The following references are of record in the file of this patent:

#### UNITED STATES PATENTS

| Number    | Name           | Date           |
|-----------|----------------|----------------|
| 1,365,606 | Seymour-Jones  | Jan. 11, 1921  |
| 1,370,709 | Smith          | Mar. 8, 1921   |
| 1,555,389 | Stevens        | Sept. 29, 1925 |
| 1,563,943 | Adams et al.   | Dec. 1, 1925   |
| 1,659,371 | Merrill        | Feb. 14, 1928  |
| 2,006,364 | Morse          | July 2, 1935   |
| 2,353,877 | Chollar        | July 18, 1944  |
| 2,427,765 | Chollar        | Sept. 23, 1947 |
| 2,427,836 | Chollar et al. | Sept. 23, 1947 |
| 2,467,213 | Luaces         | Apr. 12, 1949  |
| 2,500,573 | Rockoff        | Mar. 14, 1950  |